

## UNITED STATES PATENT OFFICE

2,186,850

## COLOR PHOTOGRAPHY

Gustav Wilmanns, Wolfen, Kreis Bitterfeld, and Adolf Sieglitz, Frankfort-on-the-Main-Hochst, and Alfred Fröhlich, Dessau in Anhalt, Germany, assignors, by mesne assignments, to Agfa Anseco Corporation, Binghamton, N. Y., a corporation of Delaware

No Drawing. Application February 20, 1937,  
Serial No. 126,842. In Germany February 27,  
1936

14 Claims. (Cl. 95-6)

Our present invention relates to the art of color photography.

One of its objects is a process of producing photographic color pictures by means of dyestuff components. A further object is the provision of novel photographic materials used for producing the photographic color pictures. Further objects will be seen from the detailed specification following hereafter.

10 It is known that in the production of photographic pictures in color there may be used with advantage as dyestuff components a number of compounds which are characterized by a particularly active methylene group. For example, methylphenylpyrazolone has been proposed for the color development. This body forms a red dyestuff picture on the parts where there is a silver precipitate produced by development of a silver picture with para-dimethylaminoaniline. If for the production of color pictures the silver antidiazotate process according to German Patent 561,867 corresponding to U. S. Patent 1,963,197 or similar processes working with diazonium compounds are used, one obtains by coupling with acetic acid ester anilides yellow dyestuff pictures.

In addition to the aforesaid bodies, however, there are compounds which, notwithstanding that they have a reactive methylene group, are not suitable intermediate products for obtaining photographic color pictures since they do not yield dyestuffs and for that reason cannot be used as components for color development or in certain cases for the treatment with diazo-compounds. Examples of these ineffective bodies are fluorene, benzofluorene, indene, dihydioresorcinol, hydroxythionaphthene, diphenylmethane and cyclohexanol.

This invention is based on the observation that the methylene group in such compounds may be made particularly active if the body is converted into an oxalic acid ester derivative of the compound or derivative thereof. These oxalic acid ester derivatives, which provisionally may be regarded as compounds of the following structure:



50 behave in the photographic color processes as do

the bodies having the highly reactive methylene groups referred to above. For example, the oxalic acid ester of fluorene of the following formula



yields when used as dyestuff component in color development a red dyestuff picture of particularly pure tint when dimethylaminoaniline is used as a developer, the oxalic acid ester of indene



on the other hand giving a blue picture by a like treatment. In processes in which diazo-bodies are used the oxalic acid ester 2:3-benzofluorene yields a yellow dyestuff when coupled with  $\beta$ -naphthylene diazotate. By the application of these oxalic acid ester derivatives for the purpose of color photography the number of color tints obtainable by the multi-color photographic processes is considerably expanded and enriched.

These oxalic acid ester derivatives may be added either to the treatment baths or to the layer material before exposure, if desired, to the gelatin before or during the preparation of the emulsion, in a form stable to diffusion, either in the most finely dispersed form as insoluble compounds or after they have been converted into suitable substitution products which are soluble in water as described in U. S. Patent applications Ser. No. 10,704 filed March 12, 1935, Ser. No. 72,718 filed April 4, 1936, Ser. No. 90,726 filed July 15, 1936, and Ser. No. 94,340 filed August 5, 1936.

From these emulsions there may be cast a single layer material or a multi-layer material having the layers either on one or on both sides of a support. The support may either consist of a transparent material as for instance Celluloid, 50

cellulose-acetate or of a light-reflecting material, as for instance paper.

The following examples serve to illustrate the invention:

- 5 1. An exposed silver halide emulsion layer is developed by means of a developer consisting of a solution of 3 grams of p-aminodimethyl-aniline and 1000 cc. of a 3% soda-solution to which are added 1.5 grams of the oxalic acid ester of flu-
- 10 orene.

15



A red color picture is obtained.

- If in the same developer the oxalic acid ester of fluorene is replaced by the oxalic acid ester of indene there is obtained a blue dyestuff image.

- 20 2. An exposed silver halide emulsion layer is developed, fixed and the silver image transformed into an azo-dyestuff image by means of the diazo-compound of  $\beta$ -naphthylamine. If this diazo silver image is immersed into a weak acetic acid solution of the oxalic acid ester of 2,3-benzo-fluorene, a yellow azo-dyestuff image is obtained.

- 25 What we claim is:
- 30 1. A light-sensitive silver halide emulsion containing as a dyestuff component for color forming development a compound containing a methylene group activated by substitution of one hydrogen atom thereof by a radical having the following formula:



wherein R is an alkyl radical.

- 40 2. A light-sensitive silver halide emulsion containing as a dyestuff component for color forming development a compound containing a methylene group, said compound being per se insufficiently reactive to form a dye by color forming development but being activated by substitution of one hydrogen atom of the methylene group by a radical having the following formula:



45 50 wherein R is an alkyl radical.

3. A light-sensitive silver halide emulsion containing as a dyestuff component for color forming development a compound containing a methylene group activated by substitution of one hydrogen atom thereof by a radical having the following formula:



- 60 60 wherein R is an alkyl radical, said dyestuff component containing in addition a radical which renders it fast to diffusion.

4. A light-sensitive silver halide emulsion containing as a dyestuff component for color forming development a compound containing a methylene group selected from the group consisting of fluorene, benzofluorene, indene, dihydroresorcinol, hydroxythionaphthene, diphenylmethane and cyclohexanol, in which the methylene group is activated by substitution of one hydrogen atom by a radical of the following formula:



75 75 wherein R is an alkyl radical.

- 5 5. A color forming developer comprising an aromatic amino developing agent and a compound containing a methylene group activated by substitution of one hydrogen atom thereof by a radical of the following formula



wherein R is an alkyl radical.

- 10 6. A color forming developer comprising an aromatic amino developing agent and a compound containing a methylene group, said compound being per se insufficiently reactive to form a dye by color forming development but being activated by substitution of one hydrogen atom of the methylene group by a radical of the following formula



15 wherein R is an alkyl radical.

- 20 7. A color forming developer comprising an aromatic amino developing agent and a compound selected from the group consisting of fluorene, benzofluorene, indene, dihydroresorcinol, hydroxythionaphthene, diphenylmethane and cyclohexanol, in which the methylene group is activated by substitution of one hydrogen atom by a radical of the following formula



25 wherein R is an alkyl radical.

- 30 8. The method of developing a colored image in a gelatino-silver halide photographic layer which method comprises coupling the developing product of an aromatic amino developing compound simultaneously with the development of a silver image in the layer with a compound containing a methylene group activated by substitution of one hydrogen atom thereof by a radical having the following formula



35 45 wherein R is an alkyl radical.

9. A light-sensitive silver halide emulsion containing as a dyestuff component for color formation a compound containing a methylene group activated by substitution of one hydrogen atom thereof by a radical having the following formula



50 55 wherein R is an alkyl radical.

10. A light-sensitive silver halide emulsion containing as a dyestuff component for color formation a cyclic compound containing a nuclear methylene group activated by substitution of one hydrogen atom thereof by a radical having the following formula



60 65 wherein R is an alkyl radical.

11. A light-sensitive silver halide emulsion containing as a dyestuff component for color forming development a cyclic compound containing a nuclear methylene group activated by substitution of one hydrogen atom thereof by a radical having the following formula



70 75 wherein R is an alkyl radical.

12. A light-sensitive silver halide emulsion as defined in claim 1 wherein the compound containing the methylene group is indene and wherein the radicle activating said methylene group is



13. A light-sensitive silver halide emulsion as defined in claim 1 wherein the compound containing the methylene group is fluorene and

wherein the radicle activating said methylene group is



14. The developer defined in claim 7 wherein the developing agent is p-dimethyl-amino-aniline.

GUSTAV WILMANNS.  
ADOLF SIEGLITZ. 10  
ALFRED FRÖHLICH.